

## UNITED STATES PATENT OFFICE

1,955,039

## CONCENTRATING MANGANESE ORES

Arthur John Weinig and Robert Emmett Cuthbertson, Golden, Colo., assignors to Cuban-American Manganese Corporation, New York, N. Y., a corporation of Delaware

No Drawing. Application November 19, 1930,  
Serial No. 496,815

3 Claims. (Cl. 209—166)

Our invention relates to improved processes of concentrating oxide manganese ores by gravity concentration and/or flotation concentration, and comprises the use of a novel reagent combination for recovering the oxide manganese minerals as a froth concentrate, and in some cases treating the crude manganese ores to a calcining roast before concentration of any kind is attempted, which preliminary calcination has been found to greatly improve the concentration and recovery 10 of the manganese minerals on difficult ores which require such treatment.

We have discovered that in the flotation concentration treatment of oxide manganese ores, 15 the use of a reagent combination of fish oil soap together with an aromatic hydrocarbon compound or mixture of hydrocarbon compounds such as dipentene, xylene, and the light oil fraction from coal tar distillation, is very effective in 20 recovering the oxide manganese minerals as a froth concentrate.

We have further discovered that the oxide manganese minerals may be successfully recovered by the flotation concentration treatment by using a 25 reagent combination of fish oil soap together with an aliphatic hydrocarbon, or mixtures of aliphatic hydrocarbon compounds, such as kerosene and crude petroleum, or kerosene and crude oil. Some 30 cheap by-product hydrocarbon compound, such as gas-oil, may be substituted for kerosene in our reagent combination.

We have also discovered that on certain difficult ores containing normally a large quantity of colloidal ore slime, calcining the crude ore, prior 35 to concentration, greatly assists in the subsequent gravity concentration and/or flotation concentration. This calcining may be accomplished by heating the crude ore preferably at a temperature of about 600° C. for about fifteen minutes, although temperatures above or below 600° C. may 40 be used for longer or shorter times than fifteen minutes. As a further benefit derived from calcination, non-oxide manganese ores are converted to oxide which can then be recovered by 45 our specific concentration methods.

We have found that a considerable variation 50 in the quantities of reagents may be employed in the flotation of the manganese minerals. Of course from an economic standpoint it is preferred to use the smallest quantities of reagents which will yield the best commercial results. As concrete examples, fish oil soap has been employed in amounts ranging from five to fifty pounds per ton of ore treated by flotation, and hydrocarbons 55 have been used in amounts ranging from one to

thirty pounds per ton of ore treated by flotation. The amounts of the two classes of reagents depend on the character of the ore; whether it contains a large or small percentage of manganese minerals; whether it contains a high or low percentage of colloidal slime, etc. 60

As an example illustrative of our improved processes, we give the following description without however restricting ourselves to the specific details set forth: 65

Raw or mine-run ore would first be dry crushed to a convenient size, say  $\frac{1}{2}$  inch. This step may be accomplished by any of the machines or combination of machines commonly employed for dry ore crushing. 70

The crushed ore may then be introduced into a rotary kiln for calcining if the character of the ore makes this treatment necessary before concentration, or the crushed ore may be concentrated without this calcining step. If calcining 75 is done on the ore, it will be heated up to 750° C. for a suitable period of time. (Lower calcining temperatures are usually found sufficient.) This calcining of the ore drives off combined water from the manganese minerals thus raising 80 their specific gravity advantageously for gravity concentration; it also converts non-oxide manganese minerals to oxides, and furthermore it destroys colloidal slime by dehydration, which slime would otherwise be detrimental to success- 85 ful concentration by gravity or flotation methods.

After the mine-run ore has been reduced by dry crushing and in some cases further treated by calcination, it is then ready for concentration proper. Sizing by screens may then be employed 90 as a first step in the concentration process. The coarse sizes from this screen sizing would then be fed into jigs where a jig concentrate of coarse manganese minerals is produced together with a jig tailing which would be further treated by re-grinding and flotation. The fines from the initial screen sizing could be passed over concentrating tables for recovery of a table concentrate of fine manganese minerals, while the table tailing would join the jig tailing for regrinding and flotation. 100 Both the jig and table tailings would be ground in ball or rod mills to a fineness sufficient to liberate the finest manganese minerals from the gangue constituents of the ore, the fineness of grind depending on the degree of intergrowth of 105 such minerals with gangue, but ranging generally from 48 to 200 mesh.

This grinding would be done in the presence of water and the resulting ore water mixture is called a pulp. This pulp containing a requisite 110

amount of water is then fed into a flotation machine where it is agitated with introduction of finely divided air. Fish oil soap is added which produces a froth. A hydrocarbon compound or 5 mixture of hydrocarbon compounds is also added to act as a slime controlling or slime depressing reagent. In addition to froth production by fish oil soap and slime depression by hydrocarbon compounds, both of these two types of reagents 10 are instrumental in causing the manganese minerals to attach themselves to air bubbles which are constantly rising to the surface of the pulp. Under these conditions the manganese minerals collect in a layer on top of the pulp and may be 15 then removed and recovered.

We have found it better practice to add the fish oil soap and the hydrocarbons separately, but usually to the same place in the flotation circuit which may consist of rougher cells and cleaner 20 cells. We have also found it convenient to add the fish oil soap in the form of a water mixture which may be prepared by adding fish oil soap to water and then heating until a fluid mixture is obtained.

25 It is understood, of course, that other reagents may be used in addition to fish oil soap and hydrocarbon compounds for specific reasons in the flotation of the oxide manganese minerals without in any way sacrificing the essential advantages 30 of our invention.

By our method of treatment higher recoveries 35 of the manganese minerals can be obtained in the treatment of oxide manganese ores than was possible by older methods, thereby making it feasible to treat ores that otherwise would not be commercially available. By our improved methods it is also possible to concentrate by flotation oxide

manganese ores which have hitherto been regarded as non-amenable to the flotation concentration process.

Our improved processes for concentration of manganese ores comprise essentially the use of 80 a novel reagent combination of fish oil soap and hydrocarbons for recovery of the oxide manganese minerals in the form of a froth concentrate, and also when necessary, calcination of the crude manganese ores as a pretreatment for 85 gravity concentration and/or flotation.

We claim as our invention:—

1. The process of concentrating oxide manganese ores which consists in subjecting said 90 ores in the form of a pulp of finely-divided material to a froth flotation operation with agitation and aeration in the presence of a reagent produced by the combined interaction of fish oil soap, crude oil and kerosene.

2. The froth flotation reagent combination for 95 treating oxide manganese ores comprising fish oil soap and dipentene mixed with a light oil fraction from coal tar distillation.

3. Those steps in the process of concentrating 100 oxide manganese ores in the form of a pulp of finely-divided material to a froth flotation operation with agitation and aeration in the presence of a reagent produced by the combined interaction of fish oil soap, crude oil and kerosene which consist in first adding the fish oil soap to said aqueous ore pulp to produce a froth and then adding the crude oil and kerosene thereto, said crude oil and kerosene controlling and depressing the slime therein.

110

ARTHUR JOHN WEINIG.

ROBERT EMMETT CUTHERBERTSON.

40

115

45

120

50

125

55

130

60

135

65

140

70

145

75

150